

# UNITED STATES PATENT OFFICE.

RALPH E. MYERS, OF EAST ORANGE, NEW JERSEY, ASSIGNOR TO WESTINGHOUSE LAMP COMPANY, A CORPORATION OF PENNSYLVANIA.

## PROCESS OF MAKING FILAMENTS.

1,180,066.

Specification of Letters Patent. Patented Apr. 18, 1916.

No Drawing.

Application filed December 5, 1910. Serial No. 595,672.

To all whom it may concern:

Be it known that I, RALPH E. MYERS, a citizen of the United States, and a resident of East Orange, in the county of Essex and State of New Jersey, have invented a new and useful Improvement in Processes of Making Filaments, of which the following is a specification.

My invention relates to processes of pre-10 paring and treating metallic filamentary structures, such as are used in electric incan-15 descent lamps, and it has for its object the provision of a process whereby filaments containing molybdenum, tungsten, tantalum and similar highly refractory metals, may be rendered more ductile and tenacious than they are previous to the application of the treatment.

The process consists in first producing the20 material of which the filament is composed in filament or wire form according to any known or desired process, as by mixing a finely divided metal, such as molybdenum, tungsten, tantalum, or other refractory25 metal with a binder, squirting this paste through a die, and then treating it to car-30 bonize and remove the binder and to sinter the finely divided particles together, the final step or steps of the treatment pref-35 erably being accomplished by passing an electric current through the material. A further treatment is then applied to the material which consists of again heating it for a short period, as by passing current35 through it, but to a lower temperature than that employed for sintering purposes, this further treatment being applied in the air and apparently serving to anneal the ma-40 terial, as it is thereby rendered much more ductile and tenacious than it is previous to the application thereto of such treatment. Wire produced according to this process may be handled and manipulated at pleasure without breakage, and because of its45 high fusing point, it is particularly suitable for use in making anchors or supports for tungsten and other metallic filaments, especially when composed of molybdenum.

In practising the present process, I prefer50 to carry it on continuously, as by passing the filamentous paste, as it leaves the die, through, or in engagement with, a series of electrical terminal devices by means of which gradually increasing amounts of cur-

rent may be applied to the moving material 55 in order to give it the ordinary treatment, and whereby an annealing current or tem-perature may also be applied to the material after it has been sintered. The cooling of the material is preferably effected grad-60 ually. After the filament has been thus treated, it may sometimes be desirable to reduce its diameter, as by drawing it through a die or swaging it by impact, or by any known or desired means, and then 65 to re-anneal it by heating in the air and cooling, the reducing in diameter, heating and cooling treatments being successively applied until the filament has been reduced to the desired diameter and rendered suffi-70 ciently ductile and tenacious. After each reduction in the diameter of the filament it will usually be found advantageous to first heat it to a higher temperature than that used for the first annealing and then to re-75 duce its temperature to approximately that used for the first annealing.

Prior attempts to anneal bodies of tung-80 sten, molybdenum and similar metals have always included the step of inclosing the metal to be annealed in a vacuum or in a non-oxidizing atmosphere. I have discov-85 ered that the annealing process may be carried out in the air and without special pre-cautions against oxidation, except that the heating, as indicated above, must continue for a short time only. My process, as set-90 forth above, is therefore superior to previ-ously known processes in simplicity as well as efficiency. Furthermore, I have discov-95 ered the rather surprising fact that, when refractory metals are annealed in the pres-ence of air or other oxidizing medium, the resulting products are less brittle and more uniform in structure than the products pro-100 duced by annealing in a vacuum or in an inert atmosphere. For example, molybde-num wire when annealed in an atmosphere of hydrogen is brittle in spots, while the same variety of wire, annealed in the same 105 manner but in the presence of air, is entirely uniform and thoroughly annealed. The reasons for this improvement are somewhat obscure. It may be that carbon is removed by oxidation, and such decarbonizing may account for the improved quality of the product. This, however, is not certain, and I do not wish to be limited by any definite

theory of chemical or physical action. It is a fact, however, that the beneficial results set forth above are not obtained in the absence of an oxidizing atmosphere and are obtained in the presence of such an atmosphere.

The foregoing treatment produces a coating of oxid upon the surface of the metal, which may be removed, if desired, by heating in hydrogen after the annealing step.

I claim as my invention:

1. The process of manufacturing fine ductile filaments from wire of refractory conducting material which consists in drawing the wire through a die and subsequently heating the product in the presence of oxygen.
2. The process of manufacturing fine ductile filaments from wire of refractory conducting material which consists in drawing the wire through a die, heating the product to an annealing temperature in the presence of air and allowing the same to cool.
3. The process of manufacturing fine ductile filaments from wire of refractory conducting material which consists in successively drawing the wire and heating it in an oxidizing atmosphere until a product of the desired diameter is obtained.
4. The combination with the step of increasing the ductility of a wire of refractory conducting material by mechanical working, of the step of increasing the ductility of the wire by heating in the presence of air.

5. The combination with the step of increasing the ductility of a wire of refractory material by drawing through a die, of the step of increasing the ductility of the product by heating in the presence of air.

6. The combination with the step of increasing the ductility of a body of refractory conducting material by successive mechanical workings, of the step of increasing the ductility of the product by successive heating in the presence of air, the two steps being applied alternately.

7. The process of manufacturing formed articles of refractory electrically-conducting material which consists in successively subjecting the said material to mechanical working and to heat applied in an oxidizing atmosphere.

8. The process of manufacturing formed articles of refractory electrically-conducting material which comprises mechanically working the said material and heating the product in an oxidizing atmosphere.

In testimony whereof, I have hereunto subscribed my name this 23rd day of November, 1910.

RALPH E. MYERS.

Witnesses:

GEORGE P. SCHOLL,  
CHARLES E. KELLY.